

## UNITED STATES PATENT OFFICE

AUGUST HARTMANN, OF BARMEN, GERMANY, ASSIGNOR TO AMERICAN BEMBERG CORPORATION, OF NEW YORK, N. Y.

PROCESS FOR THE PRODUCTION OF ARTIFICIAL SILK BY THE COPPER OXIDE AMMONIA STRETCH SPINNING PROCESS

No Drawing. Application filed November 13, 1928, Serial No. 319,189, and in Germany November 15, 1927.

It is known to produce copper oxide ammonia silk by circulating a portion of the precipitating liquid and replacing the other portion by fresh precipitating liquid, compare American Letters Patent 957,460. In this case, however, the precipitating space was divided up into two parts in such a manner that first of all, the fresh precipitating liquid alone was effective in the upper part immediately under the spinning nozzle, and the fresh portion and the portion which had already been used, and which was to be used again, then arrived mixed together at the lower portion and only there were effective. The spinning apparatus for carrying out this process required two conductors for the precipitating liquids.

Recently only one precipitating liquid and one spinning apparatus have been used with only one conductor. In this case, the whole quantity of precipitating liquid was always supplied fresh and the used precipitating liquid allowed finally to run away to waste after the copper and ammonia had been recovered. The whole quantity of liquid to be employed has then to be continually renewed, which entails considerable expense.

I have now discovered that it is not necessary to work always with fresh precipitating liquid even when employing only one precipitating liquid, but the latter may be used again, if the content of the copper and ammonia are maintained below a certain limit. This discovery enables a considerable saving in the precipitating liquid to be effected in the process according to the present invention.

According to my invention, in which only one circulating precipitating liquid is employed, a portion of this liquid is withdrawn during the circulation and freed from copper and ammonia by substantially the same amount as these have been dissolved in the whole precipitating liquid by the precipitating process. Whether the amount of precipitating liquid withdrawn can be introduced again, after being worked-up, into the circulating liquid, or whether it must be replaced by fresh precipitating liquid, depends upon the kind of spinning solution

and the method of working-up employed. If a cellulose solution produced with the aid of copper hydrate as one of the starting materials is employed, the portion of precipitating liquid worked-up may again be introduced into the circulating liquid, since it is possible in this case, by distilling off the ammonia, the copper then precipitating out in the form of copper hydrate, to recover again the ammonia and the copper without further constituents remaining behind in the worked-up liquid. If, on the other hand, the spinning solution is produced by the use of basic copper sulphate, it is then not possible to so work-up the portion of the precipitating solution withdrawn that no constituents remain behind, and for this reason, the portion withdrawn cannot again be conducted into the circulating liquid. In this case, it is necessary to replace the portion withdrawn by fresh precipitating liquid. A considerable saving of precipitating liquid is still effected, however, since hitherto the whole of the precipitating liquid was allowed to run to waste even if it was worked-up.

If the portion of the precipitating liquid withdrawn is worked-up until it can be used again, then the quantity of the liquid withdrawn itself depends on how far the working-up treatment should proceed. This is illustrated in the following example, in which  $\frac{2}{3}$  of the precipitating liquid is employed again without further treatment, while  $\frac{1}{3}$  of the liquid is worked-up.

At the commencement of the precipitating process, 1 cubic-metre of precipitating liquid contains 1.05 kilograms of ammonia and 0.12 kilograms of copper in the form of copper hydrate. At the end of the precipitating process, the ammonia content amounts to 1.4 kilograms and the copper content to 0.16 kilograms. Accordingly, 0.35 kilograms of ammonia must be removed, for example by boiling, from 1 cubic-metre of precipitating liquid in circulation. The corresponding quantity of copper thereupon precipitates out by itself. The portion of precipitating liquid withdrawn,  $\frac{1}{3}$  of a cubic-metre, now contains 0.47 kilograms of

ammonia, while 0.35 kilograms are to be removed. Thus, 0.12 kilograms of ammonia may remain in that portion of the precipitating liquid which is withdrawn. If it so happens that all the ammonia is to be driven off from the portion withdrawn from circulation, the quantity to be withdrawn is then reduced accordingly.

What I claim is:—

- 10 1. In the production of artificial silk by the copper oxide ammonia process, the steps comprising recirculating a stream of precipitating liquid containing copper oxide ammonia, withdrawing a portion of such recirculated liquid, removing copper and ammonia from said portion and returning it to the recirculated stream.
- 20 2. In the production of artificial silk by the copper oxide ammonia process, the steps comprising recirculating a stream of precipitating liquid containing copper oxide ammonia, withdrawing a portion of said stream, removing ammonia from said portion by heating and separating the copper precipitated thereby, and returning said treated portion to the recirculated stream.
- 30 3. In the production of artificial silk by the copper oxide ammonia process, the steps comprising recirculating a stream of precipitating liquid containing copper oxide ammonia, maintaining the concentration of the recirculated stream constant by withdrawing a portion of it and removing sufficient ammonia and copper from said portion by heating and separating the copper precipitated to dilute the recirculated stream to the desired concentration and returning such treated portion to the recirculated stream.
- 40 4. A process for the production of artificial thread by the copper oxide ammonia process, comprising recirculating a precipitating liquid containing copper oxide ammonia, withdrawing a portion of said liquid, heating said portion to liberate substantially all of the ammonia and separating the copper precipitated thereby, and reintroducing said portion into the recirculated liquid.
- 50 5. A process for the production of artificial thread by the copper oxide ammonia process, comprising recirculating a precipitating liquid containing copper oxide ammonia, removing about a third of said precipitating liquid, treating said removed third to remove ammonia substantially equivalent to the amount dissolved by a single circulation of the precipitating liquid, separating the copper precipitated during

said treatment and re-introducing the treated liquid into the re-circulating liquid.

6. A process for the production of artificial thread by the copper oxide ammonia process, comprising recirculating a precipitating liquid containing copper oxide ammonia, withdrawing a portion of said liquid containing more copper oxide and ammonia than is dissolved in said liquid during a single circulation of the same, heating said portion to remove sufficient ammonia to reduce the remainder of said portion to a concentration such that when it is returned to the re-circulating liquid the mixture will have the desired concentration, separating the copper precipitated during the heating, and re-introducing said treated portion to the re-circulating liquid.

7. In a process for producing cuprammonium filaments, the steps of extruding the filaments into a bath of precipitating liquid, and when the ammonia content of the precipitating liquid approaches 1.4 kilograms per cubic meter, removing approximately 0.35 kilograms of the ammonia by withdrawing a portion of the precipitating liquid and heating it, the liquid so treated being then returned to the main body of the said bath.

8. In a process for producing cuprammonium filaments, the steps of extruding the filaments into a bath of precipitating liquid, and when the ammonia content of the precipitating liquid approaches 1.4 kilograms per cubic meter and the copper content approaches 0.16 kilograms per cubic meter, removing approximately 0.35 kilograms of the ammonia, and the copper, by withdrawing a portion of the precipitating liquid and heating it, the liquid so treated being then returned to the main body of the said bath.

9. The process as set forth in claim 7, wherein the portion of the bath withdrawn is equivalent to one-third of the total quantity of the bath.

10. In a process for maintaining the precipitating value of a cuprammonium coagulating bath, the steps of using a bath until the ammonia content approaches 1.4 kilograms per cubic meter, withdrawing and heating a portion of the bath so that the ammonia is removed therefrom, and then returning this portion of the bath to the main portion, the portion of the bath being so selected that approximately 0.35 kilograms of ammonia per cubic meter are removed in this way.

AUGUST HARTMANN.